

## UNITED STATES PATENT OFFICE

MILTON O. SCHUR, OF BERLIN, NEW HAMPSHIRE, ASSIGNOR TO BROWN COMPANY, OF BERLIN, NEW HAMPSHIRE, A CORPORATION OF MAINE

## MANUFACTURE OF PULP ARTICLES

No Drawing. Application filed February 20, 1930. Serial No. 430,145.

This invention relates to the manufacture of pulp articles, and more particularly to those comprising a multiplicity of plies or webs of interfeltd fiber which are superposed in wet condition after formation on suitable web-forming instrumentalities, such as cylinder or wet machines, then dried, and, if desired, impregnated with suitable waterproofing material, such as pitch. An example of pulp articles of this class is so-called fiber conduit, which is made by winding a wet web of pulp on a mandrel to the desired wall thickness, then removing the mandrel from the resulting tube, drying the tube, and impregnating the tube with pitch. Such conduit is serviceable for use in housing underground electric wiring systems and in piping water or other fluids.

One of the important factors incident to the manufacture of such articles is the use of a stock or furnish leading to wet multi-ply products which are capable of being dried at a high rate of speed without undergoing splitting between laminations, and in the case of wet tubes, which do not go "out of round" during the drying operation. Another important factor is the use of a stock or furnish which leads to a dry multi-ply product of sufficient porosity to undergo impregnation, as with molten pitch, with uniformity and rapidity.

In the commercial production of articles such as described, and more particularly fiber conduit, it is important to attain the foregoing desiderata with comparatively inexpensive raw materials. Heretofore it has been the practice to use as the stock or furnish for forming the web approximately equal proportions of virgin ground-wood and highly beaten sulphite pulp screenings. The function of the screenings is to provide strength, and of the ground-wood to provide porosity so that the conduit may be satisfactorily impregnated with pitch. When screenings are used alone in well-beaten condition, the tubes made therefrom are liable to become warped and wrinkled during drying, and the walls shrink to such a hard, dense condition that they are incapable of undergoing impregnation in any commercially feasible

way. When the screenings are used alone in practically unbeaten condition, there is very poor bonding between plies, and the tubes are liable to split during drying. When ground-wood is used alone, although the shrinkage of the tubes on drying is very low and their porosity high, they are deficient in strength and, because of the poor cohesion between plies, they are liable to split during drying.

Waste paper stock is much less expensive than virgin ground-wood, so that were it possible to use waste papers with satisfaction in lieu of ground-wood, a very substantial saving in the cost of raw material would ensue. In the past, attempts to do this have resulted in failure, because tubes made from furnishes containing waste papers invariably undergo splitting during the drying operation and are of low strength. Apparently the waste paper stock interferes to such an extent with the realization of bonding between plies that the shrinkage strain during drying overcomes such bonding as is obtained and causes separation of the plies. I have discovered that if ground charcoal is used as one of the components of the furnish, waste papers may be used in place of virgin ground-wood, without danger of splitting during the drying operation, and further that the dry tubes may be impregnated with greater facility and with a higher pitch to fiber ratio than were the charcoal omitted. This discovery is highly significant from a commercial standpoint, as it enables a high reduction in the cost of the raw material. I have further found that if the screenings or other long-fibered stock is used either entirely or partly in the form of gel, i. e., hydrated as for the manufacture of glassine paper or even to a greater extent, a further reduction in cost may be effected, as less screenings and still more waste papers may be used. At the same time, a material increase in strength of tubes is realized when gel is used, so that strength need not be sacrificed when waste papers are substituted for the virgin ground-wood.

Various furnishes falling within the purview of the present invention may be used, the waste papers running to as high as 70%.

of the total solids of the furnish, the ground charcoal being present to the extent, of say 5% to 15%, and virgin cellulose fiber in beaten condition constituting the rest of the solids. The waste papers employed may include newspapers, magazines, cardboard, and other wastes which contain a large proportion of ground-wood.

A specific furnish which has been found to give eminently satisfactory results was made up of the following components:

|                                      | Per cent |
|--------------------------------------|----------|
| Screenings (thoroughly beaten) ----- | 42 1/2   |
| Waste papers (well-pulped) -----     | 42 1/2   |
| 15 Ground charcoal -----             | 15       |

When such a pulp furnish was formed into tubes and the tubes then dried, it was found that shrinkage in tube length was materially less than in the case of the furnishes heretofore used. This, too, is a highly advantageous feature, especially in a mill where large scale production is carried on.

Another eminently satisfactory furnish in which even more waste papers was employed comprised the following components:

|                                       | Per cent |
|---------------------------------------|----------|
| Waste papers (well-pulped) -----      | 65       |
| Long-fibered pulp (well-gelled) ----- | 25       |
| 30 Ground charcoal -----              | 10       |

The long-fibered pulp may be screenings, kraft, or sulphite stock, screenings such as obtained from sulphite pulp being preferred because of their low cost. The beating of such stock is preferably carried out in a stone-roll beater, with the roll so adjusted that at the end of, say, ten to fifteen hours, the fibers are thoroughly fibrillated and in highly gelatinized condition.

40 The procedure preferably followed in producing the furnish is to condition each component independently and then to mix the components. Such a procedure is preferable, in that each component is conditioned with greater facility in the absence of the others. For instance, the presence of the waste papers in the beater in which gelatinization of the virgin fiber is effected is objectionable in that the waste papers impede gelatinization of the virgin fiber and consume energy without undergoing much gelatinization. The virgin fiber alone is hence thoroughly gelled as, say, a 6% stock suspension, as already described.

55 The waste papers alone are preferably initially broken up by the use of a so-called "hog," whereupon the disintegrated mass is placed in a beater wherein it is well pulped with water to form, say, a 6% stock suspension. The ground charcoal is thoroughly mixed with water to produce a 10% suspension. The three suspensions are then delivered in the desired proportions into a tank wherein they are intimately mixed to produce a suspension of, say, about 6 1/2% solids content.

60 This mixture is diluted to the usual solids

content, say about 1/2%, in passing to the cylinder machine or other web-forming mechanism.

For the manufacture of tubes which are not to be impregnated, for instance tubes which are to serve as corks upon which sheet material such as paper may conveniently be wound into rolls, a furnish containing a larger proportion of long-fibered pulp, such as kraft, may be used to advantage. All of the long-fibered component may be well-beaten or it may be partly well-beaten and partly well-gelled, as this leads to tubes of high strength. The fact that the tubes may be lower in porosity is immaterial in such case, as subsequent impregnation of the tubes is not effected. A typical furnish for such tubes may comprise the following components:

|                                  | Per cent |
|----------------------------------|----------|
| Waste papers (well-pulped) ----- | 50       |
| Kraft pulp (well-gelled) -----   | 20       |
| Kraft pulp (well-beaten) -----   | 20       |
| Ground charcoal -----            | 10       |

While the furnishes hereinbefore given were described as being specifically applicable to tube or conduit manufacture, nevertheless these furnishes or others having the general composition of the present invention are advantageous in the manufacture of other multi-ply products, such as sheets, which are stripped from the make-up roll of a cylinder machine, then dried, and, if desired, impregnated with waterproofing or other materials. They may also be used in the manufacture of pulp articles, irrespective of whether the articles are composed of laminations or not, as they are inexpensive as compared with the usual furnishes of similar strength. Thus fiber furnishes such as described may be used to advantage in the manufacture of pressed pulp articles and the like, where cheapness of furnish, strength of product, and ease of drying are desirable. They are, however, of maximum advantage in the manufacture of multi-ply pulp articles to be impregnated with waterproofing materials of the character of pitch, where comparatively slight changes in the composition of the stocks heretofore used have in the past given rise to much spoilage in product, particularly when drying and impregnating equipment were operated at normal capacities.

This application is a continuation in part of my application Ser. No. 382,202, filed July 30, 1929, wherein I have disclosed, among other things, a furnish for the manufacture of pulp articles containing waste paper stock and charcoal. I do not herein claim broadly the use of charcoal in cellulose pulp furnishes intended for manufacture into articles, and more particularly into multi-ply articles to be impregnated with media such as asphalt, as this broader phase of invention is claimed in application Serial

No. 382,202. On the contrary, all the claims herein presented involve the use of waste paper stock as an essential ingredient of the pulp furnish or the article made therefrom.

5 I claim:

1. A furnish for the manufacture of pulp articles, comprising an aqueous suspension of a mixture of waste paper stock, ground charcoal and beaten, long-fibered stock.
- 10 2. A furnish for the manufacture of pulp articles, comprising an aqueous suspension of a mixture of waste paper stock, ground charcoal, and highly gelatinized, virgin, long-fibered pulp.
- 15 3. A furnish for the manufacture of pulp articles, comprising an aqueous suspension of a mixture of solids comprising up to about 70% waste paper stock, about 5% to 15% ground charcoal, and virgin cellulose fiber in beaten condition.
- 20 4. A furnish for the manufacture of pulp articles, comprising an aqueous suspension of a mixture of solids comprising the following components in substantially the proportions given:

|                                            | Per cent |
|--------------------------------------------|----------|
| Waste papers in well-pulped condition      | 65       |
| Long-fibered pulp in well-gelled condition | 25       |
| 30 Ground charcoal                         | 10       |

5. A process which comprises beating virgin cellulose pulp in water to effect its gelatinization, pulping waste papers in water, forming an aqueous suspension of ground charcoal, and then intimately mixing all these materials to produce a furnish for forming into pulp articles.

6. A pulp article formed of bonded-together webs of interfelted fiber throughout which ground charcoal is distributed, the fibers comprising both waste paper fiber and beaten virgin fiber.

7. A pitch-impregnated tube made up of bonded-together convolutions comprising waste papers, ground charcoal, and beaten, virgin, cellulose fiber.

8. A furnish for the manufacture of pulp articles, comprising an aqueous suspension of a mixture of waste paper stock, ground charcoal, and cellulose pulp beaten or hydrated to a slimy consistency.

In testimony whereof I have affixed my signature.

MILTON O. SCHUR.